

## UNITED STATES PATENT OFFICE

2,516,640

## HYDRAULIC FLUIDS

Charles W. Montgomery and William I. Gilbert,  
Oakmont, and Robert E. Kline, Penn Township,  
Allegheny County, Pa., assignors to Gulf  
Research & Development Company, Pitts-  
burgh, Pa., a corporation of Delaware

No Drawing. Application November 6, 1947,  
Serial No. 784,512

16 Claims. (Cl. 252—79)

1

This invention relates to hydraulic fluids, and more particularly to fluids for use in hydraulically operated apparatus, such as brake mechanisms, fluid flywheels, shock absorbers, control mechanisms and similar hydraulically operated equipment.

Various fluids have previously been proposed for use in hydraulic systems as hydraulic power transmission media or the like. In a great number of the previously proposed fluids, there have been many disadvantages attendant to their use, such as corrosive and degrading effects of such fluids on metal and rubber parts of the hydraulic equipment, a tendency towards volatilization at operating temperatures, lack of sufficient lubricating properties, etc.

It is an object of this invention, therefore, to provide a hydraulic fluid which overcomes the disadvantage of many of the prior art materials.

It is a further object of this invention to provide hydraulic fluids which have general utility under variable operating conditions.

These and other objects are accomplished by the present invention wherein we provide as a hydraulic fluid for hydraulic equipment a liquid comprising a substantially neutral ester of a monohydric alcohol and the mixture of acids obtained by the oxidation with gaseous oxygen of an aqueous alkaline slurry of a finely divided carbonaceous material selected from the group consisting of coal and coke obtained by the carbonization of coal at temperatures below 700° C. For convenience, the acids described above are hereinafter referred to as coal acids.

We have found that the substantially neutral monohydric alcohol esters of the mixture of coal acids described above provide excellent hydraulic fluids which are characterized by general utility under a wide variety of operating conditions. These esters may be readily and cheaply prepared, and therefore are an attractive source of hydraulic fluids.

As has been stated, the acids used in the preparation of our new hydraulic fluids are obtained by the oxidation with gaseous oxygen of an aqueous alkaline slurry of a finely divided carbonaceous material selected from the group consisting of coal and coke obtained by the carbonization of coal at temperatures below 700° C. Suitable coals comprise anthracite, bituminous, sub-bituminous, lignite and other low grade coals. Suitable cokes are those produced by the carbonization of a coal at a temperature below 700° C. in a manner known to the art. If the cokes are produced at temperatures in excess of 700° C., they

2

become graphitic and unsuitable for the production of coal acids in a satisfactory yield.

The following is an example of the preparation of the coal acids.

5 Finely ground bituminous coal, alkali, such as sodium hydroxide, and water are mixed in a nickel-lined autoclave equipped with a turbo-mixer and with means for heating and cooling the charge. The amount of alkali used is in excess 10 of that required completely to neutralize all of the coal acids formed in the oxidation process. By way of example, the proportion of the ingredients may be 15 pounds of coal, 15 gallons of water and 45 pounds of caustic soda. The 15 charge is heated and then oxygen is bubbled therethrough. The temperature of the charge is maintained from 200° to 300° C. at a total pressure of from 500 to 1200 pounds per square inch. The reaction is exothermic and the temperature is maintained within the limits stated by cooling, such as by passing water through an internal cooling coil in the autoclave. The oxidation is continued until all of the carbonaceous material of the coal passes into solution and usually requires between 2 and 3 hours. Half of the carbon of the coal is oxidized to organic acids and the remainder to carbon dioxide. At the completion of the oxidation the charge is cooled to about 110° C. and is discharged from the autoclave. The ash of the coal, which is largely unattacked, is removed by filtering through a filter press.

The filtered product is an alkaline solution containing the sodium salts of the organic acids obtained by the oxidation of the coal. Enough sulfuric acid is added to this solution to liberate the free acids. Any insoluble material appearing after acidification with sulfuric acid is removed by filtering. The free coal acids obtained 40 are water-soluble and may conveniently be obtained from their solution in water by extraction with a water-immiscible organic solvent. For example, methyl ethyl ketone may be used for this purpose, since in the presence of the sodium sulfate produced by the acidification with sulfuric acid, methyl ethyl ketone is water-immiscible. The extract phase may then be transferred to a still for recovery of the bulk of the solvent, and the product remaining in the still may then be fed 45 to a vacuum rotary drier for removal of the remainder of the solvent. For convenience in subsequent handling, the dried product may be ground to a fine powder in a pebble mill.

The product obtained appears to be a mixture 55 of aromatic acids. This mixture is a free-flowing

yellow powder which is hygroscopic and substantially completely soluble in water. The average molecular weight of the acids is 250 and the average equivalent weight is 80. Accordingly, the average number of carboxyl groups per molecule is somewhat more than 3. The exact nature of the acids is unknown, but they are believed to contain tri- and tetra-carboxylic benzene acids, as well as acids having a more complex nucleus than the benzene ring.

In order to obtain the hydraulic fluids of our invention, the coal acids as obtained above are esterified with a monohydric alcohol to produce substantially neutral esters. Esterification may conveniently be carried out by refluxing 6 moles of the alcohol with 1 mole of the coal acids for several hours while continuously adding small amounts of anhydrous hydrogen chloride as a catalyst. Water is continuously removed from the reaction vessel until the theoretical amount of separated water indicates that reaction is complete. At this point any excess of the alcohol is allowed to distill out of the reaction vessel. Other methods of esterification may be employed, as will be understood in the art.

A wide variety of monohydric alcohols may be employed for the esterification. For example, the alkanols, particularly the straight chain alkanols containing up to 20 carbon atoms, such as methyl, ethyl, propyl, butyl, amyl, hexyl, octyl, decyl, lauryl, myristyl, palmityl and eicosyl alcohols yield excellent products. Branched chain alkanols such as isopropyl alcohol, 2-ethyl-hexyl alcohol, and the individual by product alcohols obtained from the methanol synthesis may also be employed. Other monohydric alcohols which may be employed are the unsaturated aliphatic alcohols such as allyl alcohol, crotonyl alcohol, oleyl alcohol and the like. Alicyclic and aromatic monohydric alcohols such as cyclohexanol and benzyl alcohol are also suitable. Mixtures of monohydric alcohols may also be employed, particularly the mixture of alcohols obtained by the reduction of coconut oil fatty acids and known commercially as "Lorol," the mixture of higher molecular weight alcohols obtained as a product in the synthesis of methanol from carbon monoxide and hydrogen, as well as the mixture of alcohols obtained as a by product in the synthesis of hydrocarbons from carbon monoxide and hydrogen. A preferred subgroup of monohydric alcohols comprises the straight chain aliphatic alcohols containing from 4 to 12 carbon atoms.

If desired, the esters obtained as indicated above may be treated with lime and an adsorbent such as fuller's earth in order to purify the crude product. For example, in one such treatment the esters are stirred with 4 per cent by weight of fuller's earth and 4 per cent by weight of lime at a temperature of 150° to 200° C., and are then filtered.

Representative properties of some of the esters of this invention are shown in the following table:

The esters of the coal acids obtained as described hereinabove present a number of properties making them eminently suitable as hydraulic fluids. The high initial boiling points and extremely low vapor pressures of the esters, even at elevated temperatures, render any loss of these hydraulic fluids by vaporization under service conditions extremely remote. As a matter of fact, the esters of the coal acids cannot be distilled in appreciable amounts by ordinary distillation techniques and can only be partially fractionated by molecular distillation. The esters are very stable, particularly with respect to oxidation. They also have high viscosity indexes, high flash points and excellent lubricating properties. In general, the lower straight chain alkanol esters of the coal acids, including the octyl ester, have pour points sufficiently low to give them general utility as hydraulic fluids. For those monohydric alcohol esters having a relatively high pour point, such as the lauryl ester, the addition of solvents or diluents in the proportions hereinafter disclosed serves very effectively to lower the pour points without materially affecting the desirable properties of the esters. By reason of the fact that the esters are anticorrosive, they may safely be used in contact with the metal parts of hydraulic equipment without requiring the addition of a corrosion inhibitor. The esters have a high specific gravity and are therefore excellently adapted for use as fluid flywheels. In brief, the esters of the coal acids present an aggregation of properties in a single material which renders them particularly suitable for general use as hydraulic fluids, and in addition, it is unnecessary to add corrosion inhibitors and lubricants which are normally required to be added to prior art hydraulic fluids.

Although we have disclosed the use of the esters of the coal acids as hydraulic fluids by themselves, diluents and/or solvents may be added to the coal esters to produce homogeneous hydraulic fluids. When a diluent is used it will ordinarily be present in an amount from about 5 to about 50 per cent by weight on the esters of the coal acids depending upon the particular requirements, such as whether a light or heavy grade of fluid is required for a particular application. Although the esters of coal acids are soluble in a wide variety of solvents, it is preferred to use relatively non-volatile solvents boiling in the kerosene range or above as diluents of the esters in our hydraulic fluids. Thus the lower aliphatic alcohols, such as methanol, ethanol and propanol, and the low boiling hydrocarbons, such as benzene and toluene, are not desirable as diluents. Typical solvents which may be used as diluents are (1) the glycol ethers including the mono-butyl ether of ethylene glycol, the monoethyl ether of ethylene glycol, the methyl ether of ethylene glycol monoacetate, the butyl ether of diethylene glycol and the diethyl ether of ethylene glycol; and (2) hydrocarbon solvents such as light lubricating oils, gas oils, kerosene and the like.

| Ester             | Initial B. P., ° C.<br>at 760 mm. | Sp. Gr.             | Vis., SSU at<br>100° F. | Vis., SSU at<br>210° F. | VI  | Pour Pt.,<br>° F. |
|-------------------|-----------------------------------|---------------------|-------------------------|-------------------------|-----|-------------------|
| n-Butyl (crude)   | greater than 271                  | 1.094 at 130°/60° F | 2,479                   | 130                     | 76  | -----             |
| n-Butyl (treated) | greater than 271                  | 1.143 at 60°/60° F  | 10,210                  | 360                     | 92  | -----             |
| n-Octyl (crude)   | greater than 380                  | 1.0420 at 60°/60° F | 1,654                   | 117                     | 95  | 0                 |
| n-Octyl (treated) | greater than 380                  | 1.0420 at 60°/60° F | 1,820                   | 123                     | 94  | 0                 |
| n-Lauryl (crude)  | greater than 366                  | 0.9659 at 60°/60° F | 1,218                   | 116                     | 115 | +55               |
| n-Lauryl          | greater than 366                  | 0.9659 at 60°/60° F | 1,267                   | 120                     | 116 | +60               |

<sup>1</sup> Treated with fuller's earth and lime as disclosed in the preceding paragraph.

The following data illustrate some of the properties of the coal acid esters containing diluents. Data for the ester per se are included for comparison.

| Composition                                              | Specific Gravity, 60°/60° F. | Viscosity, SUS |         | Viscosity Index | Pour Point, °F. |
|----------------------------------------------------------|------------------------------|----------------|---------|-----------------|-----------------|
|                                                          |                              | 100° F.        | 210° F. |                 |                 |
| n-Octyl Ester                                            | 1.041                        | 1,605          | 114     | 94              | -10             |
| 80% Octyl Ester<br>20% Ethylene Glycol Monoethyl Ether   | 1.018                        | 266            | 53.8    | 122             | less than -70   |
| 80% Octyl Ester<br>20% Diethylene Glycol Monobutyl Ether | 1.023                        | 504            | 65.9    | 105             | -65             |

The hydraulic fluids of the present invention, whether comprising the esters of the coal acids alone or in combination with a diluent as described above, may be used as fluid power and transmission media in any of the common hydraulic systems wherein power is transmitted from an actuatable element to an actuated element by means of a fluid, the most common form of such a system comprising a pair of variable volume chambers with connecting conduit means, the chambers and the conduit means being filled with a fluid hydraulic power transmission medium. The hydraulic fluids of the present invention may also be used in analogous equipment in which power transmission is not the primary purpose as, for example, in power absorption systems, such as damping mechanisms, shock absorbers and the like.

What we claim is:

1. The process which comprises transmitting power by means of a liquid containing a substantially neutral ester of a monohydric alcohol and the mixture of acids obtained by the oxidation with gaseous oxygen of an aqueous alkaline slurry of a finely divided carbonaceous material selected from the group consisting of coal and coke obtained by the carbonization of coal at temperatures below 700° C.

2. The process of claim 1, wherein the monohydric alcohol is an alkanol containing up to 20 carbon atoms.

3. The process of claim 1, wherein the monohydric alcohol is an alkanol containing from 4 to 12 carbon atoms.

4. The process of claim 1, wherein the monohydric alcohol is butyl alcohol.

5. The process of claim 1, wherein the monohydric alcohol is octyl alcohol.

6. The process of claim 1, wherein the monohydric alcohol is lauryl alcohol.

7. The process of claim 1, wherein the finely divided carbonaceous material is bituminous coal.

8. The process of claim 1, wherein the liquid contains additionally a relatively non-volatile diluent boiling at least in the kerosene range.

9. A homogeneous hydraulic fluid comprising (1) a substantially neutral ester of a monohydric alcohol and the mixture of acids obtained by the oxidation with gaseous oxygen of an aqueous alkaline slurry of a finely divided carbonaceous material selected from the group consisting of coal and coke obtained by the carbonization of coal at temperatures below 700° C., and (2) a relatively non-volatile diluent therefor boiling at least in the kerosene range and being present in an amount of from 5 to 50 per cent by weight.

10. The fluid of claim 9, wherein the diluent is a glycol ether.

11. The fluid of claim 9, wherein the diluent is a hydrocarbon solvent.

12. The fluid of claim 9, wherein the monohydric alcohol is a straight chain alkanol containing from 4 to 12 carbon atoms.

13. The fluid of claim 9, wherein the monohydric alcohol is butyl alcohol.

14. The fluid of claim 9, wherein the monohydric alcohol is octyl alcohol.

15. The fluid of claim 9, wherein the monohydric alcohol is lauryl alcohol.

16. The fluid of claim 9, wherein the finely divided carbonaceous material is bituminous coal.

CHARLES W. MONTGOMERY.

WILLIAM I. GILBERT.

ROBERT E. KLINE.

#### REFERENCES CITED

40 The following references are of record in the file of this patent:

#### UNITED STATES PATENTS

Number Name Date  
45 2,390,258 Katz et al. Dec. 4, 1945

#### FOREIGN PATENTS

Number Country Date  
50 429,175 Great Britain May 20, 1935  
454,628 Great Britain Oct. 5, 1936

#### OTHER REFERENCES

Chemical Abstracts, vol. 40 (1946), page 5223.  
Beilstein: vol. IX, 4th ed., page 1010, and the  
55 1st supplement thereto on page 443.